# EUROPEAN PATENT SPECIFICATION

(11) **EP 3 141 643 B1**
(45) Date of publication and mention of the grant of the patent: **08.06.2022**
(21) Application number: 16188260.0
(22) Date of filing: 12.09.2016
(51) Int. Cl.: D03D 15/567, D03D 27/08

(54) **TERRY ARTICLE WITH SYNTHETIC FILAMENT YARNS AND METHOD OF MAKING SAME**
POLFADENARTIKEL MIT SYNTHETISCHEN GARNEN UND VERFAHREN ZUR HERSTELLUNG DAVON
ARTICLE EN TISSU EPONGE COMPRENANT DES FILS CONTINUS SYNTHETIQUES ET SON PROCEDE DE FABRICATION

(30) Priority: 10.09.2015 IN 3474MU2015; 26.09.2015 US 201514866916
(43) Date of publication of application: 15.03.2017
(73) Proprietor: Welspun India Limited, Mumbai 400013 (IN)
(72) Inventor: Goenka, Dipali, 400013 Mumbai (IN)
(74) Representative: Avidity IP

(56) References cited:
- EP-A1- 2 534 987
- US-A- 3 030 691

## Description

### TECHNICAL FIELD

The present disclosure relates to articles formed from terry fabrics with filaments yarns and methods of making same.

### BACKGROUND

Terry fabrics have a wide range of end uses. More common examples are towels, bath robes, rugs, top of the bed fabrics, bath mats, and seat covers. Terry fabrics include ground warp yarns, weft yarns interwoven with warp yarns, and pile yarns that define pile loops on one or both sides of the fabric. Terry fabrics are cut to size and hems or selvedges formed along the edges define the shape of the article. Terry fabric design takes into consideration end-use performance requirements and aesthetics. Design features that impact fabric properties and therefore contribute to performance of the fabric during use include fiber type, yarn type, yarn count, pile height, pile density, ground fabric structure, and fabric weight. Optimizing fabric structure for the end-use requirements is difficult and is not always a predictable endeavor. It is known from such document as US 3030691 (Law Marvin A) and EP 2534987 (Tricol Japan Co Ltf) to provide terry fabrics in which pile loops are provided with natural and synthetic yarns which are globally treated to vary the length of pile loops but ensuring and maintain proper presentation of the variation in height for best effect has not been considered.

### SUMMARY

There is a need for an article formed from a terry fabric that includes natural and synthetic yarns that also has improved cushion and unique visual features. An embodiment of the present disclosure is a terry article that includes a ground component including a plurality of ground warp yarns and a plurality of weft yarns, and a pile component disposed on at least one of a lower side and an upper side of the ground component. The pile component includes a first plurality of pile loops that extend away from the ground component along a vertical direction. The first plurality of pile loops are formed from a first set of pile yarns comprised of natural fibers and further define a first pile height. The pile component also includes a second plurality of pile loops that extend away from the ground component in the vertical direction. The second plurality of pile loops are formed from a set of continuous filament thermoplastic yarns and define a second pile height that is less than the first pile height.

The terry article of the present invention includes a ground component including a plurality of ground warp yarns and a plurality of weft yarns interwoven with the plurality of ground warp yarns. The weft yarns and the ground warp yarns each include at least one of a natural fiber and a synthetic fiber. The ground component includes a first side and a second side opposed to the first side along a vertical direction. The terry articles also includes a first pile component disposed on the first side that also includes a plurality of piles, and a second pile component disposed on the second side and that includes a plurality of piles. The plurality of piles the first pile component includes: 1) a first plurality of pile loops that extend away from the ground component along the vertical direction, the first plurality of pile loops formed from a first set of pile yarns comprised of natural fibers, the first plurality of pile loops including a first pile base located at the ground component, a first pile end spaced apart from the first pile base, and a first pile height that extends from the first pile base to the first pile end along the vertical direction; and 2) a second plurality of pile loops that extend away from the ground component in the vertical direction, the second plurality of pile loops formed from a set of continuous filament thermoplastic yarns, the second plurality of pile loops including a second pile base at the ground component, a second pile end spaced apart from the second pile base, and a second pile height that extends from the second pile base to the second pile end along the vertical direction. The second pile height is less than the first pile height.

Another embodiment of the present disclosure is terry article. The terry article includes a ground component including a plurality of ground warp yarns and a plurality of weft yarns interwoven with the plurality of ground warp yarns. The weft yarns and the ground warp yarns each include at least one of a natural fiber and a synthetic fiber. The ground component includes a first side and a second side opposed to the first side along a vertical direction. The terry article also includes a first pile component disposed on the first side. The first pile component includes a first plurality of pile loops that extend away from the ground component along the vertical direction. The first plurality of pile loops are formed from a first set of pile yarns comprised of natural fibers. The first plurality of pile loops includes a first pile base located at the ground component, a first pile end spaced apart from the first pile base, and a first pile height that extends from the first pile base to the first pile end along the vertical direction. The terry article includes a second pile component disposed on the second side. The second pile component includes a second plurality of pile loops that extend away from the ground component in the vertical direction. The second plurality of pile loops are formed from a set of continuous filament thermoplastic yarns, the second plurality of pile loops including a second pile base at the ground component, a second pile end spaced apart from the second pile base, and a second pile height that extends from the second pile base to the second pile end along the vertical direction. The second pile height is less than the first pile height.

The present invention also includes a method of making a terry article. The includes the step of weaving a pile fabric to include a ground component and a pile component disposed on at least one of an upper side and a lower side of the ground component. The weaving step forms the pile component with a first plurality of pile loops formed from natural fiber yarns and a second set of pile loops formed from continuous filament thermoplastic yarns. The method includes, after the weaving step, thermally treating the pile fabric such that the continuous filament thermoplastic yarns shrink, thereby decreasing a pile height of the second plurality of pile loops relative to a pile height of the first plurality of pile loops.

### BRIEF DESCRIPTION OF THE DRAWINGS

The foregoing summary, as well as the following detailed description of illustrative embodiments of the present application, will be better understood when read in conjunction with the appended drawings. For the purposes of illustrating the present application, there is shown in the drawings illustrative embodiments of the disclosure. It should be understood, however, that the application is not limited to the precise arrangements and instrumentalities shown.
Figure 1 is a top view of a terry article according to an embodiment of the present disclosure.
Figure 2 is schematic cross-sectional view of the terry article taken along line 2-2 in Figure 1.
Figure 3 is a detailed sectional view of a portion of the terry article shown in Figure 2.
Figure 4 is a top view of a terry article according to another embodiment of the present disclosure.
Figure 5 is a top view of a terry article according to another embodiment of the present disclosure.
Figure 6 is a top view of a terry article according to another embodiment of the present disclosure.
Figure 7 is a top view of a terry article according to another embodiment of the present disclosure.
Figure 8 is a process flow diagram illustrating process steps in the manufacture the terry article illustrated in Figures 1-7.

### DETAILED DESCRIPTION OF ILLUSTRATIVE EMBODIMENTS

As shown in Figures 1 and 2, the terry article 10 includes a ground component 30 and at least one pile component. The pile component includes a first set of pile loops formed from natural yarns and a second set of pile loops formed from continuous filament thermoplastic yarns. The finishing process creates pile height differential between the first set of pile loops and the second set of loops. The pile height differential can create a visually observable texture or pattern in the terry article 10. Furthermore, improved cushion profiles are possible by designing the terry article to have different pile heights in different locations on the article 10. Embodiment of the present disclosure include several different pile configurations including first and second loops with a height differential. The different pile configuration include: a) a pile component on only one side of the article that includes the first set of pile loops and the second set of loops; b) a pile component both sides of article that includes the first set of pile loops and the second set of loops; and c) a first pile component including the first set of pile loops disposed on a first side of the article and a second pile component that includes the second set of loops disposed on the other side of the terry article.

The description and figures illustrate a towel article formed from a terry fabric as one example. However, terry articles--products made with or including terry fabrics--can include, but are not limited to, towels, bath robes, rugs, top of the bed fabrics, bath mats, and seat covers. The terry articles as described herein are suitable for home-uses, e.g. for products in bath or kitchen uses, commercial uses, such towels designed for hotels, hospitality business, healthcare and restaurants, and/or industrial uses for cleaning or wiping of spills in industrial settings.

Continuing with Figure 1, the terry article 10 includes opposed ends 12 and 14 spaced apart along a longitudinal direction 2, and side edges 16 and 18 that extend from the end 12 to end 14 along the longitudinal direction 2. The longitudinal direction 2 can be referred to as the machine direction or warp direction. The side edges 16 and 18 are spaced apart with respect to each other along a lateral direction 4 that is perpendicular to the longitudinal direction 2. The ends 12 and 14 and side edges 16 and 18 collectively define a towel perimeter, which in turn defines a size and shape of the terry article. The article 10 also includes a face 20 and a face 22 opposed to the face 20 along a vertical direction 6 that is perpendicular to the longitudinal and lateral directions 2 and 4, respectively. The terry article 10 has a length L that extends from end 12 to end 14 along the longitudinal direction 2 and a width W that extends along the lateral direction 4. As illustrated, the terry article length L is greater than the width W so as to define shape of a bath towel or hand towel. The dimensions of the terry article 10 can defined during manufacturing to any particular size. For instance, the terry article 10 can be hand towel.

Continuing with Figure 1 and 2, the terry article 10 includes ground component 30 and at least one pile component. In illustrated embodiment, the terry article 10 has an upper pile component 60 along a face 20 of the article 10 and a lower pile component 160 along a back 22 of the article 10. In some instances, the terry article 10 includes only one pile component on either the face 20 or back 22. The ground component 30 includes an upper side 32 and a lower side 34 spaced from the upper side along the vertical direction 6. The upper pile component 60 can project away from the upper side 32 of the ground component 30 along the vertical direction 6 in a first direction 8a. The lower pile component 160 can project from the lower side 34 along the vertical direction 6 in a second direction 8b that is opposite to the first direction 8a. The terry article ends 12 and 14 include hems 24a and 24b, respectively. The side edges 16 and 18 can include hems or selvages 26a and 26b, respectively. The terry article 10 can also include one or more optional borders 28 that extend across the width W or the length L of the terry article 10. For example, the terry article 10 shown in Figure 1 includes a first border 28a and a second border 28b.

As illustrated in Figure 1, the upper pile component 60 can extend across a majority of the article face 20. Specifically, the upper pile component 60 extends from one border 28a to the opposite border 28b along the longitudinal direction 2, between border 28a and end 12, and also between border 28b and end 14. The upper pile component also extends from one hem 26a at side edge 16 to the opposing hem 26b at side edge 18 along the lateral direction 4. The upper pile component 60 therefore defines substantial portion of the face 20 of the terry article 10. Accordingly, the upper pile component 60 includes a plurality of pile loops (up to all of the pile loops) located on the upper side 32 of the ground component 30. In addition, the lower pile component 160 may extend along one or both of longitudinal and lateral direction s 2 and 4 on the lower side 34 of the ground component 30. As shown, the lower pile component 160 corresponds to the upper pile component 60 such that lower pile component 160 defines a substantial portion of the back 22 of the terry article 10. Accordingly, the lower pile component 160 includes a plurality of pile loops, up to all of the pile loops, on the lower side 34 of the ground component 34. The upper pile component 60 may be referred to as a first pile component and the lower pile component 160 may be referred to as a second pile component.

The ground component 30 includes a plurality of ground warp yarns 40 and a plurality of weft yarns 42 interwoven with the plurality of ground warp yarns 40. The ground component 30 may defined by a number of woven structures. Exemplary woven structures for the ground component 30 include, but are not limited to, 1×1 plain weave, 2×1 rib weave, 2x2 rib weave, or 3x1 rib weave. As further explained below, the ground warp and weft yarns each comprise one or more of natural fiber and a synthetic fiber. For instance, each ground warp yarns may be natural fiber yarns, synthetic fiber yarns, or a blended natural and synthetic fiber yarns.

The ground warp yarns 40 can be formed from any number of fiber types. For instance, the ground warp yarns can be natural fiber yarns, synthetic yarns, natural and synthetic blended yarns. Synthetic yarns with good moisture absorbency and/or retention properties may be used in some instances as the ground warp yarns. The natural fiber yarns may include primarily cotton fibers, flax, bamboo, hemp, or other natural fibers. Natural and synthetic blended yarns can include blends of cotton and polyethylene terephthalate (PET) staple fibers, cotton and polylactic acid (PLA) staple fibers, and cotton and polypropylene (PP) staple fibers. The present disclosure is not limited to cotton blends. Other natural and synthetic blends include cotton and staple microfibers. Additional natural and synthetic blends include cotton and staple fibers with complex cross-sectional shapes. In another example, the natural and synthetic blended yarns can include cotton fibers in a core-spun construction with a synthetic filament comprising the core. Synthetic yarns may include rayon fibers (e.g. Modal, Lyocell), microfiber staple fibers, or blends of PET and polyamide microfibers.

The ground warp yarns 40 can be any type of spun yarn structure. For example the ground warp yarns can be ring spun yarns, open end yarns, or rotor spun yarns, or filaments In another embodiment, the ground warp yarns can be Hygrocotton ^{®} brand yarns marketed by Welspun India Limited. Furthermore, yarns can be formed as disclosed in U.S. Patent No. 8,833,075, entitled "Hygro Materials for Use In Making Yarns And Fabrics," (the 075 patent). The 075 patent is incorporated by reference into present disclosure. The ground warp yarns have a count in a range between about 984 dtex (6 Ne) to about 98 dtex (60 Ne). In one example, the ground warp yarns have a count of about 369 dtex (16 Ne). In another example, the ground warp yarns have a count of about 295 dtex (20 Ne). In another example, the ground warp yarns have a count of about 246 dtex (24 Ne). In another example, the ground warp yarns have a count of about 197 dtex (30 Ne). In another example, the ground warp yarns have a count of about 174 Dtex (34 Ne). In another example, the ground warp yarns have a count of about 148 Dtex (40 Ne). In another example, the ground warp yarns have a count of about 118 Dtex (50 Ne). In addition, the ground warp yarns can be plied yarns. In one example, the natural fiber warp yarn is 2-ply yarn. In another example, the ground warp yarns yarn is a 3 ply yarn.

The weft yarns 42 can be formed from a number of fiber types in a variety of different yarn structures. For instance, the weft yarns can be natural fiber yarns, synthetic yarns, natural and synthetic blended yarns. The ground weft yarns can be ring spun yarns, open end yarns, or rotor spun yarns, or filaments. The ground weft yarns can be Hygrocotton ^{®} brand yarns marketed by Welspun India Limited. Furthermore, yarns can be formed as disclosed the 075 patent. The weft yarns 42 can have a count in a range between about 98 Dtex (6 Ne) to about 98 Dtex (60 Ne). In accordance with the illustrated embodiment, the weft yarns 42 can be similar to the ground warp yarns described above.

Turning to Figure 3, the upper pile component 60 can be disposed on the upper side 32 of ground component 30. In accordance with the illustrated embodiment, the upper pile component 60 includes an upper first plurality of pile loops 62 that extend away from the ground component 30 in the first direction 8a. The first plurality of pile loops 62 are formed by a first set of pile yarns 64. The first plurality of pile loops 62 further define a base 66 located at the ground component 30, a pile end 68 spaced apart from the base 66 along a respective pile loop 62, and a first pile height HI that extends from the base 66 to the pile end 68. The first pile height H1 may be referred to as the upper first pile height H1.

The upper pile component 60 includes a second plurality of pile loops 72 that extend away from the ground component 30 in the first direction 8a. The second plurality of pile loops 72 are formed from a set of continuous filament thermoplastic yarns 74. The continuous filament thermoplastic yarns may be referred to as second pile yarns. Each loop 72 includes a pile base 76 at the ground component 30, a pile end 78 spaced apart from the pile base 76, and a second pile height H2 that extends from the pile base 76 to the pile end 78. The second pile height H2 may be referred to as the upper second pile height H2. The upper pile component 60 is configured such that the upper second pile height H2 is less than the upper first pile height H1 due to thermally induced shrinkage of the continuous filament thermoplastic yarns 74. In one example, the upper second pile height H2 is at about 1 mm to about 5 mm less than the upper first pile height H1. In one example, the upper second pile height H2 is at least 15 % less than the upper first pile height H1. In another example, the upper second pile height H2 is between about 15% to about 50% less than the upper first pile height H1. In another example, the upper second pile height H2 is between about 20 % to about 40% less than the upper first pile height H1. In another example, the upper second pile height H2 is between is about 20% less than the upper first pile height H1. In yet another example, the upper second pile height H2 is between is about 30% less than the upper first pile height H1. In yet another example, the upper second pile height H2 is about 40% less than the upper first pile height H1.

The upper pile component 60 includes first pile zones 80 that include the first pile loops 62 and second pile zones 82 that include the second pile loops 72. The first and second pile zones 80 and 82 can be randomly distributed across the terry article 10 such that the height differential between the first and second loops 62 and 72 creates visually perceptible texture across width W and length L of the upper pile component 60. Turning to Figures 4-7, in accordance with the illustrated alternative embodiments, the first and second pile zones 80 and 82 can define distinct shapes with respect to each other. Specifically, the first and second pile zones 80 and 82 can be configured to have one or more of a linear, curvilinear, and rectilinear shape. Figure 4 illustrates an alternative embodiment of a terry article 11a that includes a first pile zone 81a that surrounds multiple square shaped second zones 82a. In Figure 5, an alternative embodiment of a terry article 11b includes rectilinear shaped first pile zones 81b and rectilinear shaped second zones 82b. In Figure 6, in accordance with another alternative embodiment, a terry article 11c includes a first pile zone 81b that surrounds circular shaped second zones 82b. In Figure 7, an alternative embodiment of a terry article 11d includes a plurality of curvilinear shaped bands that define the first pile zones 81d and curvilinear narrow bands that define second zones 82d.

As described above, the first pile yarns 64 define the first plurality of loops. The first pile yarns 64 may include natural fibers. The natural fibers in the first pile yarns 64 can be cotton, flax, bamboo, hemp, or other natural fibers with improved moisture absorbency and retention properties. In one example, the natural fibers are cotton fibers. Furthermore, the first pile yarn can be a ring spun yarn, an open end yarn, a rotor spun yarn, or the Hygrocotton ^{®} brand yarn in accordance with the 075 patent. The first pile yarns 64 may have a count between about 984 Dtex (6 Ne) to about 98 Dtex (60 Ne). In one example, the first pile yarns 64 may have a count between 591 Dtex (10 Ne) to about 118 Dtex (50 Ne), and preferably between about 591 Dtex (10 Ne) to about 197 Dtex (30 Ne). In another example, the first pile yarns 64 may have a count between 197 Dtex (10 Ne) to about 246 Dtex (24 Ne). In one example, the first pile yarns 64 have a count of about 369 Dex (16 Ne). In another example, the first pile yarns 64 have a count of about 295 Dtex (20 Ne). In another example, the first pile yarns 64 have a count of about 246 Dtex (24 Ne). Furthermore, the first pile yarns 64 can have between about 150 and 350 turns/meter of twist, preferably between about 200 to about 300 turns/meter of twist. In addition, the first pile yarns 64 can be plied yarns. In one example the first pile yarn is 2-ply yarn. In another example, the first pile yarns 64 are 3-ply yarns. In another example, the first pile yarns 64 are 4-ply yarns.

The second pile yarns 74 include continuous filament thermoplastic yarns and define the second loops. The continuous filament yarns may include PET filaments, PLA filaments, PP filaments, or other filaments formed from thermoplastic polymers. In order to permit yarn shrinkage and this decrease pile height in the second plurality of loops, the continuous filament yarns are non-heatset yarns. Because the fiber morphology and stresses have not been fixed due to heat set processing prior to fabric formation, subsequent exposure of the continuous filament yarns in pile components to a temperature that exceeds the polymer glass transition temperature (Tg) causes the filaments to shrink along filament length and possibly radially. This in turn causes the second pile height H2 (the second pile loops) to decrease relative to the pile height H1 of the first pile loops.

In accordance with the illustrated embodiment, the continuous filament thermoplastic yarns have a count between about 295 Dtex (75) denier to about 1333 Dtex (1200 denier). In another example, the continuous filament thermoplastic yarns have a count between about 189 Dtex (170 denier) to about 589 (530), and preferably between about 222 Dtex (200 denier) to about 444 Dtex (400 denier). In one example, the continuous filament yarns have a count of about 247 Dtex (220) denier. In another example, the continuous filament yarn has a count of about 300 Dtex (270 denier). In another example, the continuous filament yarn has a count of about 367 Dtex (330) denier.

Continuing with Figure 3, the terry article 10 can also include the lower pile component 160. The lower pile component 160 is sometimes referred to as the second pile component. In accordance with the illustrated embodiment, the lower pile component 160 includes a lower first plurality of pile loops 162 that extends away from the ground component 30 in the second direction 8b. The lower first plurality of pile loops 162 are formed by a first set of pile yarns 164, which are similar to the first pile yarns 64 that form pile loops 62 in the upper pile component 60. The first plurality of pile loops 162 further define a base 166 located at the ground component 30, a pile end 168 spaced apart from the base 166 along a respective pile loop 162, and a third pile height H3 that extends from the base 166 to the pile end 168. The third pile height H3 may be referred to as lower first pile height H3. The lower pile component 160 also includes a lower second plurality of pile loops 172 that project away from the ground component 30 in the second direction 8b. The second plurality of pile loops 172 are formed from a set of continuous filament thermoplastic yarns 174 which are similar the continuous filament yarns 74 that form loops 72 in the upper pile component 60. The second plurality of pile loops 172 include a pile base 176 at the ground component 30, a pile end 178 spaced apart from the pile base 176, and a fourth pile height H4 that extends from the pile base 176 to the pile end 178. The fourth pile height referred to as the lower second pile height H4. The lower pile component 160 is configured such that the fourth pile height H4 is less than the third pile height H4 as a result of thermally induced shrinkage of the continuous filament thermoplastic yarns 174. In one example, the lower second pile height H4 is at least 15 % less than the lower first pile height H3. In another example, the lower second pile height H4 is between about 15% to about 50% less than the lower first pile height H3. In another example, the lower second pile height H4 is between about 20 % to about 40% less than the lower first pile height H3. In another example, the lower second pile height H4 is between is about 20% less than the lower first pile height H3. In yet another example, the lower second pile height H4 is between is about 30% less than the lower first pile height H3. In yet another example, the lower second pile height H4 is about 40% less than the lower first pile height H3.

The lower pile component 160 can also include or more first pile zones 180 that include the lower first pile loops 162, and one or more second pile zones 182 that include the lower second pile loops 172. The first and second pile zones 180 and 182 can be randomly distributed across the terry article 10 such that the height differential between the lower first and second pile loops 162 and 172 creates a visually perceptible texture across width W and length L of the lower pile component 160. In other embodiments, the first and second pile zones 180 and 182 can define distinct shapes with respect to each other. For example, the pile zones 180 and 182 can define one or more of linear, curvilinear, and rectilinear shapes.

A method of making a terry article according to an embodiment of the disclosure is illustrated in Figure 8. The method 200 includes yarn formation processing steps 210 for: a) ground warp yarns, b) weft yarns, c) the first pile warp yarns, and d) the second pile warp yarns. In embodiments where the terry article 10 includes upper and lower pile components 60 and 160, yarn formation 210 can includes forming additional first and second pile yarn sets for the lower pile component 160. Exemplary yarn formation phases will be described next.

During yarn formation 210, the ground warp yarns may be formed from any number of fiber types. The ground warp yarns can be formed primarily with natural fibers, natural and synthetic blended fibers, and synthetic fibers or yarns with good moisture absorbency and/or retention properties, as described above. In one example, the ground warp yarns are formed primarily from natural fibers, such as cotton.

Yarn formation 210 for the ground warp yarns can include various staple yarn spinning systems. Such yarn spinning systems may include bale opening, carding, optionally combing, drafting, roving, and yarn spinning (yarn spinning processes are not illustrated) to the desired count and twist level. In some cases, the ground warp yarns can be plied into 2-ply, 3-ply, or 4-ply configurations. After yarn spinning, the ground warp yarns are wound into the desired yarn packages for ground warp preparation step 220. In one example, ring spinning is the preferred spinning system. However, the ground warp yarns can be formed using open end spinning systems or rotor spun spinning systems. Furthermore, the spinning system may include methods to form the Hygrocotton ^{®}, as disclosed in the 075 patent. The 075 patent is incorporated by reference into present disclosure.

During yarn formation 210, the weft yarns may be formed with similar fiber types and using the same or similar yarn spinning systems used to form the ground warp yarns. As needed the weft yarns may be plied in 2-ply, 3 ply, or 4-ply configurations. Following weft yarn spinning, the weft yarns are wound onto desired packages. The wound packages are then staged for weft insertion during fabric formation steps discussed further below.

Yarn formation step 210 includes forming the upper first pile yarns 64 from natural fibers using typical yarn spinning systems. For instance, the first pile yarns 64 may formed using the same or similar process to how the warp yarns were formed. In one example, the natural fibers are cotton fibers. The first pile yarn formation steps produces pile yarns with a desired count and twist level as described above. However, it should be appreciated that the first pile yarn count and twist level can vary as needed based on the specific end use. First pile yarn formation steps may include plying the yarns into 2-ply, 3-ply, or 4-ply configurations. In addition, the first pile yarns 64 can be formed from blends of cotton and synthetic fibers, such as PET fibers. In alternative embodiments, the first pile yarns 64 are formed using other fibers, such as viscose rayon.

The second pile yarns 74 are formed via continuous filament yarn formation systems. In continuous filament yarn formation, polymer resins (such as PET, PLA, and PP) are melted and extruded through orifices at temperatures that approach the polymer melting temperature (Tm). From the orifices, the filaments may be slightly tensioned by passing over one or more godets before being wound onto a desired yarn packages. Additional bulking or texturizing steps may be included to increase the bulk and impart "false twist" to the yarns. Preferably, the continuous filament yarns 74 are not subjected to extensive heat drawing and tension during yarn formation so that the resulting filaments are not heat set (or heat set via subsequent steps prior to fabric formation). Accordingly, the second pile yarns 74 are sometimes referred to as non-heatset yarns. Non-heatset yarns can shrink if exposed to temperatures at or above the respective polymer glass transition temperature (Tg), in absence of tension applied to the yarns. As further described below, utilization of non-heatset yarns 74 to form the second pile loops and the subsequent exposure to sufficient thermal energy causes the second pile loops 72 to shrink and reduce the pile height H2, as further detailed below. Continuous filament formation steps result in continuous filament yarns 74 with the desired counts as described above.

In a method of forming terry article 10 with upper and lower pile components 60 and 160, the yarn formation step 210 may include forming lower first and second lower pile yarns, in addition to the steps of forming upper first and second pile yarns 64 and 74. Forming lower first and second pile yarns is similar to the production steps in forming the first pile yarns 64 and the second pile yarns 74.

Following the yarn formation 210, the method proceeds to a ground warp preparation step 220 and a pile warp preparation step 230. The ground warp preparation step 220 includes one or more ground warping steps, whereby the ground yarn ends are removed from their respective yarn packages, arranged in a parallel form, and wound onto a ground warp beam. The ground warp preparation step 220 also includes a sizing step where a typical sizing agent is applied to each ground warp yarn to aid in fabric formation. The ground warp preparation step 220 results in a warp beam of ground warp yarns prepared for weaving. The ground warp beam can be positioned on a mounting arm of a weaving loom so that the ground warp yarns can be drawn through the loom components, as further described below.

The pile warp preparation step 230 includes similar steps to the ground warp preparation steps--warping and sizing. In particular, pile warp preparation 230 includes warping and sizing the first pile yarns 64 (e.g. the natural fiber pile yarns). Furthermore, the pile warp preparation step 230 also includes warping and sizing a second pile warp of the continuous filament thermoplastic yarns 74 (i.e. the non-heatset yarns). Thus, the pile warp preparation step 230 results in at least two different pile warp beams: a first pile warp beam and a second pile warp beam.

For embodiments of terry articles that include upper and lower pile components 60 and 160, the pile warp preparation 230 step includes preparing four separate pile warp beams: two upper pile warp beams and two lower pile warp beams. More specifically, the pile warp preparation step 230 can include preparing warp of first pile yarns 64, e.g. natural fiber yarns. The pile preparation step 230 also includes preparing a warp of continuous filament thermoplastic yarns 74. The pile preparation step 230 also included preparing a lower first pile warp of yarns. In one example, the lower first pile yarns are natural fiber yarns that are similar to the yarns in the upper first pile warp. The pile preparation step also includes preparing a lower second warp of continuous filament thermoplastic yarns. Step 230 results in four pile warp beams, with two upper pile warp beams dedicated to forming the first and second upper loops in the upper pile component 60, and two lower pile warp beams dedicated to forming the first and second lower loops in the lower pile component 160. The ground and pile warp beams are positioned on respective mounting arms or mounting brackets proximate the weaving loom (not shown).

Continuing with Figure 8, following the ground warp and pile warp preparation steps 220 and 230, a weaving step 240 forms a pile fabric by forming the ground component 30 and the pile component on one side (or both sides) of the ground component 30 using a weaving loom designed for terry weaving. More specifically, in the weaving step 240, each ground warp yarn and pile warp yarn from the respective warp beams are drawn-in (not shown) through various components of a weaving loom, such as drop wires, heddle eyes attached to a respective harness, reed and reed dents, in a designated order as is known in the art.

After drawing-in is complete, the weaving step 240 proceeds through two phases: a ground component formation phase and a pile component formation phase. Both phases include a particular shedding motion to facilitate interweaving the weft yarns with the ground warp yarns and pile warp yarns to create the desired pile fabric construction. For instance, shedding motions can include cam shedding, dobby shedding, or jacquard shedding motions, each of which can cause the selective raising and lowering of warp ends to create an open shed for weft insertion. In one example, the weaving loom may be configured for one type of shedding motion for the ground warp yarns and another type of shedding motion for the pile warp yarns. For instance, a cam or dobby shedding motion can be used for the ground warp yarns and the jacquard shedding motions can be used for the pile warp yarns. A specific reed motion and warp take-off system is utilized to form the pile loops during the pile component phase and such a mechanism using a terry weaving loom is well known and will not be repeated here.

During the ground component phase of the weaving step 240, weft yarns are interwoven with the ground warp yarns to define the ground component or ground fabric. Exemplary ground fabric woven constructions include: a 1×1 plain weave, 2x1 rib weave, 2x2 rib weave, or 3x1 rib weave. Other woven constructions in the ground fabric are possible as well. The ground component formation phase can utilize different weft insertion techniques, including air-jet, rapier, or projectile type weft (fill) insertion techniques.

The pile component phase of the weaving step 240 includes interweaving the first pile yarns 64 (via the first warp) with the ground warp and weft yarns to create a first set of pile loops that extend away from the ground component along a vertical direction V. In addition,
pick density that is 3 or more times greater than the pick density of adjacent portions of the pile fabric. The weaving step 240 can further include weaving one or more selvedge edges along a length L of the pile fabric.

The weaving step 240 can form pile fabrics having any number of different fabric constructions. In one example, the pile fabric is formed to result in a 2-pick up to 5-pick (or more) terry weave pattern. Furthermore, the pile fabric can have a 1:1 warp order where each ground warp end is followed by a pile warp end across the width of the pile fabric. In other embodiments, the pile fabric can have a 2:2 warp order a pair of ground warp ends are followed by a pair of pile warp end across the width of the pile fabric. In one example, the pile fabric can be formed to include between about 15 to about 45 ends/cm, preferably between about 20 and 30 ends/cm. The weft or pick density can range between about 10 picks/cm to about 30 picks/cm. Preferably, the pick density is between about 15 picks/cm to about 25 picks/cm.

In embodiments with upper and lower pile components 60 and 160, the weaving step 240 further includes forming upper pile component 60 on the upper side 32 of the ground component 30 and forming the lower pile component 160 on the lower side 24 of the ground component 30. As noted above, the lower pile component 160 includes a lower first set of pile loops 162 formed from natural fiber yarns and a lower second set pile loops are formed with continuous filament thermoplastic yarns.

Following weaving step 240, the pile fabric is subjected to one or more dyeing and finishing steps 250. Dyeing and finishing steps 250 include a de-sizing step and a bleaching. The method can also include a step of applying one or more dyes to the pile fabric. Such a dyeing step may include applying reactive dyes to natural fiber yarns, and cotton yarns in particular. Either batch, semi-continuous, or continuous dyeing system can be used to apply reactive dyes the pile fabric. Other dyes can be used depending on the particular fiber blend. In other embodiments, yarns can be package died (prior to weaving).

Step 250 includes a finishing step where various chemical agents are added to pile fabric to improve or augment performance characteristics of the terry article. In one example, the pile fabric can be treated with a hydrophilic agent, such as silicones. In another example, the finishing step includes application of one or more softeners to the fabric, such as cationic softeners, non-ionic softeners, and silicones. In another example, the finishing step includes application of an antimicrobial agent to the pile fabric. Other dyes can be used depending on the particular fiber blend. In other embodiments, yarns can be package died (prior to weaving).

Step 250 includes a finishing step where various chemical agents are added to pile fabric to improve or augment performance characteristics of the terry article. In one example, the pile fabric can be treated with a hydrophilic agent, such as silicones. In another example, the finishing step includes application of one or more softeners to the fabric, such as cationic softeners, non-ionic softeners, and silicones. In another example, the finishing step includes application of an antimicrobial agent to the pile fabric.

After the dyeing and finishing step 250, a thermal treatment step 260 causes the continuous filament thermoplastic yarns, i.e. the non-heatset yarns, in respective pile components 60 and 160 to shrink. Shrinkage of the continuous filament thermoplastic yarns decreases a pile height of the second plurality of pile loops relative to the pile height of the first plurality of pile loops. According to the present invention, the thermal treatment step 260 includes advancing the pile fabric through a heating machine that exposes the pile fabric to thermal energy for a period of time that is sufficient to induce shrinkage in the non-heat set yarns. The thermal energy is sufficient to expose the pile fabric to a temperature that is greater than or equal to the glass transition temperature (Tg) of the continuous filament thermoplastic yarn. The surface temperature of the pile fabric during the thermal treatment step 260 approaches or exceeds the glass transition temperature (Tg) of the continuous filament thermoplastic yarns. For non-heatset PET filament yarns, the glass transition temperature (Tg) is between about 67 to 81 degrees Celsius. For non-heatset PLA filaments, the glass transition temperature (Tg) is between about 60 to 65 degrees Celsius. For non-heatset PP filaments, the pile fabrics are exposed to temperature between about 100 and to 130 degrees Celsius. Accordingly, the desired surface temperature of the pile fabric should fall within or exceed somewhat the stated ranges for each of the fibers mention above. It should be appreciated that any suitable thermal treatment can be used, such as, convection, steam, or infrared thermal treatments. Accordingly, the heating machine can include a convection oven, a steam oven, or an infrared oven.

During the thermal treatment step 260, the pile fabric is exposed to the desired thermal energy levels for a period of time that is sufficient to induce shrinkage in the non-heatset pile yarns. The exposure time is dependent on the dwell time of pile fabric within the heating machine, which is related to the machine speed and length of the heating zones within the heating machine. In one example, the pile fabric is advanced through the heating machine at a rate that ranges between 2.0 meters/min up to about 30 meters/min, which varies based on number heating zones.

Following the thermal treatment step 260, the method includes a cutting step 270 where the pile fabric is cut to size of one or more terry articles, such as bath towel, a hand towel, and a washcloth. Following cutting 270, additional edge binding or hems can be applied to finish the cut edges. After the cutting step, a packing step 280 places the finished terry articles in suitable packaging for shipment.

While the disclosure is described herein using a limited number of embodiments, these specific embodiments are not intended to limit the scope of the disclosure as otherwise described and claimed herein.

## Claims

1. A terry article (10) comprising:
a ground component (30) including a plurality of ground warp yarns (40) and a plurality of weft yarns (42) interwoven with the plurality of ground warp yarns, wherein the weft yarns and the ground warp yarns each include at least one of a natural fiber and a synthetic fiber, the ground component including a lower side (34) and an upper side (32) opposed to the lower side along a vertical direction (6) ; and
a pile component including 1) a first plurality of pile loops (62) that extend away from the ground component along the vertical direction, the first plurality of pile loops formed from a first set of pile yarns (64) comprised of natural fibers, the first plurality of pile loops including a first pile base (66) located at the ground component, a first pile end (68) spaced apart from the first pile base, and a first pile height (H1) that extends from the first pile base to the first pile end along the vertical direction, and 2) a second plurality of pile loops (72) that extend away from the ground component in the vertical direction, the second plurality of pile loops formed from a set of continuous filament thermoplastic yarns (74), the second plurality of pile loops including a second pile base (76) at the ground component, a second pile end spaced apart from the second pile base, and a second pile height (H2) that extends from the second pile base to the second pile end (78) along the vertical direction, the second pile height is less than the first pile height, the article **characterized in that** the article has a surface in part formed by the second pile height (H2) having the ends (78) shrunk relative to the first set of pile yarns in zones 80, 82 and relative to the remaining parts of the second pile whilst maintained in a substantially stable vertical upright direction relative to each other by respective presentation on the warp yarns and weft yarns woven together.

2. The terry article of claim 1, wherein the pile component is an upper pile component (60) that is disposed on the upper side, wherein the first plurality of pile loops is an upper first plurality of pile loops, and the second plurality of pile loops is a upper second plurality of pile loops.

3. The terry article of claim 2, further comprising a lower pile component (160) disposed on the lower side, the lower pile component including a lower first plurality of pile loops and a lower second plurality of pile loops, wherein the lower second plurality of pile loops are formed from continuous filament thermoplastic yarns.

4. The terry article of claim 1, wherein the first plurality of pile loops are randomly distributed among the second plurality of pile loops across a length and width dimension of the pile component.

5. The terry article of claim 1, wherein:
the first pile zones defines one or more of a linear shape, a curvilinear shape, and a rectilinear shape; and/or
the second pile zones defines one or more of a linear shape, a curvilinear shape, and a rectilinear shape.

6. The terry article of claims land any claim dependent thereon wherein the continuous filament thermoplastic yarns include non-heat set thermoplastic filaments.

7. The terry article of any of claims land any claim dependent thereon wherein the continuous filament thermoplastic yarns have a count in a range between about 189 dtex (170 denier) to about 589 dtex (530 denier).

8. The terry article of any of claims land any claim dependent thereon wherein the first set of pile yarns have a count in a range between about 984 dtex (6 Ne) to about 98 dtex (60 Ne).

9. The terry article of any of claims land any claim dependent thereon wherein the natural fiber of the first set of pile yarns is cotton fiber.

10. A method of making a terry article (10), the comprising the steps of:
weaving (240) a pile fabric including a ground component (30) and a pile component disposed on at least one of an upper side (60) and a lower side (160) of the ground component, such that, the pile component includes a first plurality of pile loops (62) formed from natural fiber yarns and a second set of pile loops (72) formed from continuous filament thermoplastic yarns; and
after the weaving step, thermally treating (260) the pile fabric such that the continuous filament thermoplastic yarns is subject to heat shrink adjustment, thereby decreasing a pile height (H2) of the second plurality of pile loops relative to a pile height (H1) of the first plurality of pile loops,
the method **characterized in that** the heat shrink adjustment is by surface heat treatment upon pile fabric of the article above the glass transition temperature of the continuous filament thermoplastic yarn at a rate of 2 to 30 meters per minute such that ends (78) of the second piles shrinks about the surface of the pile fabric in a substantially upright vertical direction relative to the first set of pile yarns to provide that the second pile height is less than the first pile height in the substantially upright direction from the ground component upon the warp yarns and weft yarns woven together of the ground component.

11. The method of claim 11, the continuous filament thermoplastic yarns are non-heat set yarns, wherein the thermally treating step includes advancing the pile fabric through a heating machine that exposes the pile fabric to thermal energy for a period of time that is sufficient to induce shrinkage in the non-heat set yarns.

12. The method of claim 11, wherein the thermally treating step includes exposing the pile fabric to a temperature that is greater than or equal to the glass transition temperature of the continuous filament thermoplastic yarn.

13. The method of claim 11, wherein the weaving step includes:
forming the pile component on the upper side of the ground component; and
forming a second pile component on the lower side of the ground component such that the lower pile component includes a lower first plurality of pile loops and a lower second plurality of pile loops that are formed from a second set of continuous filament thermoplastic yarns.

## Patentansprüche

1. Ein Frottee-Artikel (10) umfassend:
Eine Grundkomponente (30), umfassend eine Vielzahl von Grundkettenfäden (40) und eine Vielzahl von Schussfäden (42), die mit der Vielzahl der Grundkettenfäden verwoben sind, wobei die Schussfäden und die Grundkettenfäden jeweils mindestens eine Naturfaser und eine Synthetikfaser beinhalten und die Grundkomponente eine Unterseite (34) und eine Oberseite (32) gegenüber der Unterseite entlang einer vertikalen Richtung (6) beinhaltet; und
eine Florkomponente, umfassend 1) eine erste Vielzahl von Florschleifen (62), die sich weg von der Grundkomponente entlang der vertikalen Richtung erstrecken, die erste Vielzahl der Florschleifen, die aus einem ersten Satz von Florfäden (64) gebildet sind, die Naturfasern umfassen, die erste Vielzahl der Florschleifen beinhaltet eine erste Florbasis (66) an der Grundkomponente, ein erstes Florende (68), das räumlich von der ersten Florbasis getrennt ist, und eine erste Florhöhe (H1), die sich von der ersten Florbasis zu dem ersten Florende entlang der vertikalen Richtung erstreckt, und 2) eine zweite Vielzahl von Florschleifen (72), die sich weg von der Grundkomponente in die vertikale Richtung erstrecken, die zweite Vielzahl von Florschleifen, die aus einem Satz von kontinuierlichen thermoplastischen Filamentgarnen (74) gebildet ist, wobei die zweite Vielzahl der Florschleifen eine zweite Florbasis (76) an der Grundkomponente beinhaltet, ein zweites Florende, das räumlich von der zweiten Florbasis getrennt ist, und eine zweite Florhöhe (H2), die sich von der zweiten Florbasis zum zweiten Florende (78) entlang der vertikalen Richtung erstreckt, die zweite Florhöhe ist geringer als die erste Florhöhe, der Artikel **gekennzeichnet dadurch, dass** der Artikel eine Oberfläche hat, die teilweise durch die zweite Florhöhe (H2) gebildet wird, wobei die Enden (78) im Verhältnis zu dem ersten Satz von Florfäden in den Bereichen 80, 82 und im Verhältnis zu den verbleibenden Teilen des zweiten Florfadens geschrumpft sind, während sie durch eine entsprechende Präsentation auf den miteinander verwobenen Kettenfäden und Schussfäden in einer im Wesentlichen stabilen vertikalen aufrechten Richtung im Verhältnis zueinander bleiben.

2. Der Frottee-Artikel nach Anspruch 1, wobei die Florkomponente eine obere Florkomponente (60) ist, die an der Oberseite angeordnet ist, wobei die erste Vielzahl der Florschleifen eine obere erste Vielzahl von Florschleifen ist, und die zweite Vielzahl der Florschleifen eine obere zweite Vielzahl von Florschleifen ist.

3. Der Frottee-Artikel nach Anspruch 2, ferner umfassend eine untere Florkomponente (160), die an der Unterseite angeordnet ist, wobei die untere Florkomponente eine erste Vielzahl von Florschleifen und eine untere zweite Vielzahl von Florschleifen beinhaltet, wobei die untere zweite Vielzahl von Florschleifen aus kontinuierlichen thermoplastischen Filamentgarnen gebildet ist.

4. Der Frottee-Artikel nach Anspruch 1, wobei die erste Vielzahl von Florschleifen beliebig unter der zweiten Vielzahl von Florschleifen quer durch das Längen- und Breitenmaß der Florkomponente verteilt ist.

5. Der Frottee-Artikel nach Anspruch 1, wobei:
der erste Florbereich eine oder mehrere lineare Formen, eine kurvenlinige Form und eine geradlinige Form definiert; und/oder
der zweite Florbereich eine oder mehrere lineare Formen, eine kurvenlinige Form und eine geradlinige Form definiert.

6. Der Frottee-Artikel nach Anspruch 1 und jedem davon abhängigen Anspruch, wobei die kontinuierlichen thermoplastischen Filamentgarne nicht thermofixierte thermoplastische Filamente beinhalten.

7. Der Frottee-Artikel nach Anspruch 1 und jedem davon abhängigen Anspruch, wobei die kontinuierlichen thermoplastischen Filamentgarne eine Anzahl in einem Bereich zwischen ungefähr 189 dtex (170 Denier) bis ungefähr 589 dtex (530 Denier) haben.

8. Der Frottee-Artikel nach Anspruch 1 und jedem davon abhängigen Anspruch, wobei der erste Satz von Filamentgarnen eine Anzahl in einem Bereich zwischen ungefähr 984 dtex (6 Ne) bis ungefähr 98 dtex (60 Ne) haben.

9. Der Frottee-Artikel nach Anspruch 1 und jedem davon abhängigen Anspruch, wobei die Naturfaser des ersten Satzes von Florfäden eine Baumwollfaser ist.

10. Ein Verfahren zur Herstellung eines Frottee-Artikels (10), die folgenden Schritte umfassend:
Weben (240) eines Florgewebes, das eine Grundkomponente (30) und eine Florkomponente beinhaltet, angeordnet mindestens an einer Oberseite (60) oder einer Unterseite (160) der Grundkomponente, so dass die Florkomponente eine erste Vielzahl von Florschleifen (62) beinhaltet, die aus Naturfasergarnen gebildet sind, und einen zweiten Satz von Florschleifen (72), die aus kontinuierlichen thermoplastischen Filamentgarnen gebildet sind; und
nach dem Webeschritt, die thermische Behandlung (260) des Florgewebes, bei der die kontinuierlichen thermoplastischen Filamentgarne einer Wärmeschrumpfanpassung unterzogen werden, wodurch eine Florhöhe (H2) der zweiten Vielzahl von Florschleifen im Verhältnis zu einer Florhöhe (H1) der ersten Vielzahl von Florschleifen verringert wird,
das Verfahren **gekennzeichnet dadurch, dass** die Wärmeschrumpfanpassung eine Oberflächenwärmebehandlung am Florgewebe des Artikels oberhalb der Glasübergangstemperatur des kontinuierlichen thermoplastischen Filamentgarns bei einer Rate von 2 bis 30 Metern pro Minute ist, so dass die Enden (78) des zweiten Flors die Oberfläche des Florgewebes in einer im Wesentlichen aufrechten vertikalen Richtung im Verhältnis zum ersten Satz der Florfäden schrumpft, um dafür zu sorgen, dass die zweite Florhöhe geringer ist als die erste Florhöhe in der im Wesentlichen aufrechten Richtung von der Grundkomponente an den mit der Grundkomponente verwobenen Ketten- und Schussfäden.

11. Das Verfahren nach Anspruch 11, wobei die kontinuierlichen thermoplastischen Filamentgarne nicht thermofixierte Garne sind und wobei der thermische Behandlungsschritt den Vorschub des Florgewebes durch eine Wärmeanlage beinhaltet, die das Florgewebe für eine bestimmte Zeit der Wärmeenergie aussetzt, die ausreicht, um die Schrumpfung in den nicht thermofixierten Garnen einzuleiten.

12. Das Verfahren nach Anspruch 11, wobei der thermische Behandlungsschritt die Aussetzung des Florgewebes einer Temperatur beinhaltet, die höher oder gleich ist wie die Glasübergangstemperatur des kontinuierlichen thermoplastischen Filamentgarns.

13. Das Verfahren nach Anspruch 11, wobei der Webeschritt Folgendes beinhaltet: Bilden der Florkomponente an der Oberseite der Grundkomponente; und Bilden einer zweiten Florkomponente an der Unterseite der Grundkomponente, so dass die untere Florkomponente eine untere erste Vielzahl von Florschleifen und eine untere zweite Vielzahl von Florschleifen beinhaltet, die aus einem zweiten Satz von kontinuierlichen thermoplastischen Filamentgarnen gebildet werden.

## Revendications

1. Article en tissu éponge (10) comprenant :
un élément de fond (30) comportant une pluralité de fils de chaîne de fond (40) et une pluralité de fils de trame (42) entrelacés avec la pluralité de fils de chaîne de fond, dans lequel les fils de trame et les fils de chaîne de fond comprennent chacun au moins une fibre naturelle et une fibre synthétique, l'élément de fond comportant un côté inférieur (34) et un côté supérieur (32) opposé au côté inférieur le long d'une direction verticale (6) ; et
un élément de poil comportant 1) une première pluralité de bouclettes (62) qui s'étendent à partir de l'élément de fond le long de la direction verticale, la première pluralité de bouclettes étant formée à partir d'un premier ensemble de fils de poil (64) composés de fibres naturelles, la première pluralité de bouclettes comportant une première base de poil (66) située au niveau de l'élément de fond, une première extrémité de poil (68) espacée de la première base de poil, et une première hauteur de poil (H1) qui s'étend de la première base de poil à la première extrémité de poil le long de la direction verticale, et 2) une seconde pluralité de bouclettes (72) qui s'étendent à l'écart de l'élément de fond dans la direction verticale, la seconde pluralité de bouclettes étant formée d'un ensemble de fils thermoplastiques à filaments continus (74), la seconde pluralité de bouclettes comportant une seconde base de poil (76) au niveau de l'élément de fond, une seconde extrémité de poil espacée de la seconde base de poil et une seconde hauteur de poil (H2) qui s'étend de la seconde base de poil à la seconde extrémité de poil (78) le long de la direction verticale, la seconde hauteur de poil étant inférieure à la première hauteur de poil, l'article **caractérisé en ce que** l'article présente une surface en partie formée par la seconde hauteur de poil (H2) dont les extrémités (78) sont rétractées par rapport au premier ensemble de fils de poil dans les zones 80, 82 et par rapport aux parties restantes du second poil tout en étant maintenues dans une direction verticale vers le haut sensiblement stable les unes par rapport aux autres par une présentation respective sur les fils de chaîne et les fils de trame tissés ensemble.

2. Article en tissu éponge selon la revendication 1, dans lequel l'élément de poil est un élément de poil supérieur (60) qui est disposé sur le côté supérieur, dans lequel la première pluralité de bouclettes est une première pluralité supérieure de bouclettes, et la seconde pluralité de bouclettes est une seconde pluralité supérieure de bouclettes.

3. Article en tissu éponge selon la revendication 2, comportant en outre un élément de poil inférieur (160) disposé sur le côté inférieur, l'élément de poil inférieur comportant une première pluralité inférieure de bouclettes et une seconde pluralité inférieure de bouclettes, dans lequel la seconde pluralité inférieure de bouclettes est formée de fils thermoplastiques à filaments continus.

4. Article en tissu éponge selon la revendication 1, dans lequel la première pluralité de bouclettes est distribuée de manière aléatoire parmi la seconde pluralité de bouclettes sur une dimension de longueur et de largeur de l'élément de poil.

5. Article en tissu éponge selon la revendication 1, dans lequel :
les premières zones de poil définissent une ou plusieurs formes parmi une forme linéaire, une forme curviligne et une forme rectiligne ; et/ou
les secondes zones de poil définissent une ou plusieurs formes parmi une forme linéaire, une forme curviligne et une forme rectiligne.

6. Article en tissu éponge selon la revendication 1 et une quelconque revendication dépendante de celle-ci, dans lequel les fils thermoplastiques à filaments continus comprennent des filaments thermoplastiques non thermodurcis.

7. Article en tissu éponge selon l'une quelconque des revendications 1 et toute revendication qui en dépend, dans lequel les fils thermoplastiques à filaments continus présentent un compte compris entre environ 189 dtex (170 deniers) et environ 589 dtex (530 deniers).

8. Article en tissu éponge selon l'une quelconque des revendications 1 et toute autre revendication qui en dépend, dans lequel le premier ensemble de fils de poil présente un compte compris entre environ 984 dtex (6 Ne) et environ 98 dtex (60 Ne).

9. Article en tissu éponge selon l'une quelconque des revendications 1 et toute autre revendication qui en dépend, dans lequel la fibre naturelle du premier ensemble de fils de poil est une fibre de coton.

10. Procédé de fabrication d'un article en tissu éponge (10) comportant les étapes de :
tissage (240) d'un tissu à poil comportant un élément de fond (30) et un élément de poil disposés sur au moins l'un parmi un côté supérieur (60) et un côté inférieur (160) de l'élément de fond, de sorte que l'élément de poil comporte une première pluralité de bouclettes (62) formées à partir de fils de fibres naturelles et un second ensemble de bouclettes (72) formées à partir de fils thermoplastiques à filaments continus ; et
après l'étape de tissage, le traitement thermique (260) du tissu à poil de sorte que les fils thermoplastiques à filaments continus sont soumis à un réglage de rétraction thermique, diminuant ainsi une hauteur de poil (H2) de la seconde pluralité de bouclettes par rapport à une hauteur de poil (H1) de la première pluralité de bouclettes,
le procédé est **caractérisé en ce que** le réglage de la rétraction thermique est effectué par un traitement thermique de surface sur le tissu à poil de l'article au-dessus de la température de transition vitreuse du fil thermoplastique à filaments continus à une vitesse de 2 à 30 mètres par minute de sorte que les extrémités (78) des seconds poils se rétractent autour de la surface du tissu à poil dans une direction verticale sensiblement vers le haut par rapport au premier ensemble de fils de poil pour faire en sorte que la seconde hauteur de poil soit inférieure à la première hauteur de poil dans la direction sensiblement vers le haut à partir de l'élément de fond sur les fils de chaîne et les fils de trame tissés ensemble de l'élément de fond.

11. Procédé selon la revendication 11, les fils thermoplastiques à filaments continus sont des fils non thermofixés, dans lequel l'étape de traitement thermique comporte l'avancement du tissu à poil à travers une machine de chauffage qui expose le tissu à poil à de l'énergie thermique pendant une période de temps qui est suffisante pour induire un rétrécissement dans les fils non thermofixés.

12. Procédé selon la revendication 11, dans lequel l'étape de traitement thermique comporte l'exposition du tissu à poil à une température qui est supérieure ou égale à la température de transition vitreuse du fil thermoplastique à filaments continus.

13. Procédé selon la revendication 11, dans lequel l'étape de tissage comporte :
la formation de l'élément de poil sur le côté supérieur de l'élément de fond ; et
la formation d'un second élément de poil sur le côté inférieur de l'élément de fond de sorte que l'élément de poil inférieur comporte une première pluralité inférieure de bouclettes et une seconde pluralité inférieure de bouclettes qui sont formées à partir d'un second ensemble de fils thermoplastiques à filaments continus.
